

Patented Oct. 13, 1953

2,655,471

# UNITED STATES PATENT OFFICE

2,655,471

## CHROMIUM ELECTROPLATING

Allan E. Chester, Highland Park, Ill., assignor to  
Poor & Company, Chicago, Ill., a corporation  
of Delaware

No Drawing. Application December 21, 1951,  
Serial No. 262,899

12 Claims. (Cl. 204—51)

**1** This invention relates to new and useful chromium plating baths and to a method for electrodepositing chromium from chromium plating baths.

One of the objects of the invention is to produce new and improved chromium plating baths which have a greater chromium throwing power than ordinary chromium plating baths.

Another object of the invention is to provide new and improved chromium plating baths containing an additive which retards the liberation of chromic acid fumes.

Still a further object of the invention is to provide a new and improved method for electrodepositing chromium from chromic acid baths containing sulfuric acid. Other objects will appear hereinafter.

These objects are accomplished in accordance with this invention by electrodepositing chromium from a chromic acid-sulfuric acid bath containing a trifluoroacetic acid salt of an oxyalkylated fatty amine. The quantity of the trifluoroacetic acid salt required for the purpose of the invention is relatively small but is preferably sufficient to produce a foam blanket on the chromium plating bath and to provide greater throwing power for the chromium in the bath.

The invention will be further illustrated but is not limited by the following examples in which the quantities are stated in parts by weight unless otherwise indicated.

### Example I

To a chromic acid bath containing 33 ounces of  $\text{CrO}_3$  per gallon of aqueous solution and a ratio of  $\text{H}_2\text{SO}_4:\text{CrO}_3$  within the range of 1:100 to 1:60 there is added  $\frac{1}{2}$  milliliter of the trifluoroacetic acid salt of a soybean amine oxyethylated with approximately 10 moles of ethylene oxide, containing 20 carbon atoms in its alkyl chain and having an average molecular weight of 714 (Ethomeen S/20).

Ferrous metal articles previously plated with an alloy of zinc and copper consisting of approximately 82% zinc and 18% copper were plated with chromium out of the above described bath at the current densities customarily employed in chromium plating with excellent results.

### Example II

A chromium plating bath was prepared as described in Example I except that 52 ounces of  $\text{CrO}_3$  were employed per gallon of solution. Excellent results were also obtained in plating various types of objects in this bath.

**2**

Instead of using  $\frac{1}{2}$  milliliter of the trifluoroacetic acid salt per gallon of plating solution somewhat smaller or somewhat larger amounts may be used, preferably within the range of  $\frac{1}{4}$  to 1 milliliter of said salt per gallon of plating solution.

Although especially good results have been obtained by employing the trifluoroacetic acid salt of the oxyethylated fatty amine described in the example it will be understood that other trifluoroacetic acid salts of oxyalkylated fatty amines may be employed for the purpose of the invention.

The fatty amines are amines derived from fatty acids and normally contain 8 to 36 carbon atoms but may contain as high as 60 carbon atoms. They differ from each other in the number of carbon atoms in their alkyl groups, in the degree of saturation of the alkyl groups and in the number of alkyl groups attached to the amino nitrogen. Examples of fatty amines are those derived from soya beans, those derived from coconut oil and those derived from tallow. The oxyalkylation of these amines to produce oxyalkylated amines is effected by reacting the amines with an alkylene oxide, for example, ethylene oxide, 1,2-propylene oxide, or mixtures of ethylene oxide and 1,2-propylene oxide. The number of moles of the alkylene oxide is preferably at least 4 moles per mole of primary fatty amine, and for the purpose of the present invention the preferred products contain around 10 to 20 moles of alkylene oxide per mole of primary fatty amine. The fatty amines per se are water insoluble but oxyalkylation results in the addition of ether and hydroxy solubilizing groups to the molecule increasing the degree of water solubility and decreasing the cationic strength of the resultant material.

The invention provides a method of incorporating into chromic acid plating baths an exceedingly stable cationic wetting agent containing fluorine in its molecule. The result is a decided improvement in the chromium throwing power of the bath and in the retardation of the liberation of chromic acid fumes which are exceedingly toxic. Furthermore, the operation of the bath may be continued over relatively long periods of time due to the unusual stability of the trifluoroacetic acid salts of the oxyalkylated fatty amines in such baths.

The trifluoroacetic acid salts of the oxyalkylated fatty amines are claimed as new compounds

in my copending application, Serial No. 262,898, filed of even date herewith.

The invention is hereby claimed as follows:

1. A chromic acid plating bath for the electrodeposition of chromium containing a trifluoroacetic acid salt of an oxyalkylated fatty amine in sufficient amount to retard the liberation of chromic acid fumes from said bath.

2. A chromic acid plating bath for the electrodeposition of chromium containing a trifluoroacetic acid salt of an oxyethylated fatty amine in sufficient amount to retard the liberation of chromic acid fumes from said bath.

3. A chromic acid plating bath for the electrodeposition of chromium containing in aqueous solution 33 to 52 ounces per gallon of  $\text{CrO}_3$ , a weight ratio of  $\text{H}_2\text{SO}_4:\text{CrO}_3$  of 1:100 to 1:60 and a quantity of a trifluoroacetic acid salt of an oxyalkylated fatty amine which exhibits cationic activity in said solution, said quantity of said trifluoroacetic acid salt being sufficient to produce a foam blanket on said bath.

4. A chromic acid plating bath for the electrodeposition of chromium containing in aqueous solution 33 to 52 ounces per gallon of  $\text{CrO}_3$ , a weight ratio of  $\text{H}_2\text{SO}_4:\text{CrO}_3$  of 1:100 to 1:60 and a quantity of a trifluoroacetic acid salt of an oxyalkylated fatty amine which exhibits cationic activity in said solution, said quantity being within the range of  $\frac{1}{4}$  to 1 milliliter of said trifluoroacetic acid salt per gallon of said plating solution.

5. A chromic acid plating bath for the electrodeposition of chromium containing in aqueous solution 33 to 52 ounces of  $\text{CrO}_3$  per gallon of solution, a weight ratio of  $\text{H}_2\text{SO}_4:\text{CrO}_3$  within the range of 1:100 to 1:60 and a sufficient quantity of a trifluoroacetic acid salt of an oxyethylated fatty amine containing 10 to 20 oxyethylene groups per mole of fatty amine and having in its alkyl group 8 to 36 carbon atoms to retard the liberation of chromic acid fumes from said bath.

6. A chromic acid plating bath for the electrodeposition of chromium containing in aqueous solution 33 to 52 ounces of  $\text{CrO}_3$  per gallon of solution, a weight ratio of  $\text{H}_2\text{SO}_4:\text{CrO}_3$  within the range of 1:100 to 1:60 and a trifluoroacetic acid salt of an oxyethylated fatty amine containing 10 to 20 oxyethylene groups per mole of fatty amine and having in its alkyl group 8 to 36 carbon atoms, the quantity of said salt being approximately  $\frac{1}{2}$  milliliter per gallon of said plating solution.

7. The method of chromium plating which comprises electrodepositing chromium from a chromic acid plating bath containing a triflu-

oroacetic acid salt of an oxyalkylated fatty amine in sufficient amount to retard the liberation of chromic acid fumes from said bath.

8. The method of chromium plating which comprises electrodepositing chromium from a chromic acid plating bath containing a trifluoroacetic acid salt of an oxyethylated fatty amine in sufficient amount to retard the liberation of chromic acid fumes from said bath.

9. The method of chromium plating which comprises electrodepositing chromium from a chromic acid plating bath containing in aqueous solution 33 to 52 ounces per gallon of  $\text{CrO}_3$ , a weight ratio of  $\text{H}_2\text{SO}_4:\text{CrO}_3$  of 1:100 to 1:60 and a quantity of a trifluoroacetic acid salt of an oxyalkylated fatty amine which exhibits cationic activity in said solution, said quantity of said trifluoroacetic acid salt being sufficient to retard the liberation of chromic acid fumes from said bath.

10. The method of chromium plating which comprises electrodepositing chromium from a chromic acid plating bath containing in aqueous solution 33 to 52 ounces per gallon of  $\text{CrO}_3$ , a weight ratio of  $\text{H}_2\text{SO}_4:\text{CrO}_3$  of 1:100 to 1:60 and a quantity of a trifluoroacetic acid salt of an oxyalkylated fatty amine which exhibits cationic activity in said solution, said quantity being within the range of  $\frac{1}{4}$  to 1 milliliter of the trifluoroacetic acid salt per gallon of said plating solution.

11. The method of chromium plating which comprises electrodepositing chromium from a chromic acid plating bath containing in aqueous solution 33 ounces to 52 ounces of  $\text{CrO}_3$  per gallon of solution, a ratio of  $\text{H}_2\text{SO}_4:\text{CrO}_3$  within the range of 1:100 to 1:60 and a sufficient quantity of a trifluoroacetic acid salt of an oxyethylated fatty amine containing 10 to 20 oxyethylene groups per mole of fatty amine and having in its alkyl group 8 to 36 carbon atoms to provide greater throwing power for the chromium in said bath.

12. The method of chromium plating which comprises electrodepositing chromium from a chromic acid plating bath containing in aqueous solution 33 ounces to 52 ounces of  $\text{CrO}_3$  per gallon of solution, a ratio of  $\text{H}_2\text{SO}_4:\text{CrO}_3$  within the range of 1:100 to 1:60 and a trifluoroacetic acid salt of an oxyethylated fatty amine containing 10 to 20 oxyethylene groups per mole of fatty amine and having in its alkyl group 8 to 36 carbon atoms, the quantity of said salt being approximately  $\frac{1}{2}$  milliliter per gallon of said plating solution.

ALLAN E. CHESTER.

No references cited.